

April 11, 1961

H. G. GREIG

2,979,402

ELECTROSTATIC PRINTING

Filed July 31, 1956



INVENTOR.  
Harold G. Greig  
BY J. L. Collester

ATTORNEY

1

2,979,402

## ELECTROSTATIC PRINTING

Harold G. Greig, Princeton, N.J., assignor to Radio Corporation of America, a corporation of Delaware

Filed July 31, 1956, Ser. No. 601,221

13 Claims. (Cl. 96—1)

This invention relates to electrostatic printing and particularly, but not necessarily exclusively, to improved electrophotographic recording elements for electrostatic printing and to improved methods of electrostatic printing utilizing said improved recording elements.

An electrostatic printing process is that type of process for producing a visible record, reproduction, or copy which includes, as an intermediate step, converting a light image or electric signal into an electrostatic charge pattern on an electrically-insulating base. The process includes the conversion of the electrostatic charge pattern into a visible image by the application thereto of electrostatically-attractable particles. An electrostatic printing process using a photoconducting insulating stratum to convert a light image into an electrostatic charge pattern is described by C. J. Young and H. G. Greig in "Electrofax Direct Electrophotographic Printing on Paper," RCA Review, volume XV, No. 4, pages 469 to 484 (December 1954), hereinafter referred to as the Young and Greig publication.

A typical electrostatic printing process utilizing a photoconducting insulating stratum includes first producing a blanket electrostatic charge on the surface of the photoconducting stratum. The electrostatic charge may be stored on the surface for a time in the dark. The rate at which this stored electric charge is dissipated when the stratum is maintained in darkness is hereinafter referred to as the dark decay of the stratum. Within the period in which a substantial charge remains, a light image is focused on the charged surface, discharging the portions of the surface irradiated with light, leaving the remainder of the surface in a charged condition, and thereby forming an electrostatic image thereon. The electrostatic image is rendered visible by applying to the electrostatic image a developer substance, such as a pigmented thermoplastic resin powder, which is held electrostatically to the charged areas of the surface. The visible image thus formed may be fixed directly to the surface, for example, by fusing the image thereto.

One type of recording element usable in the foregoing electrostatic printing process comprises a cellulosic sheet coated with a particulate photoconductor dispersed in an electrically-insulating, film-forming vehicle, for example, ordinary paper coated with particulate photoconducting white zinc oxide dispersed in a silicone resin. Such recording elements produce satisfactory prints if they are stored at normal or above normal humidity for a substantial period of time just prior to use. However, poor prints result if the element is stored just prior to use in a below normal humidity. Generally, the lower the humidity the poorer the print. It is believed that the reason for such poor results is that the paper backing becomes non-uniformly more insulating at lower humidities. In such condition, the electric field resulting from the blanket electrostatic charge appears non-uniformly across the backing and the photoconducting stratum instead of uniformly across only the photoconducting stratum. This greater distance, and non-uniform field

2

strengths, produce poorer results. This humidity sensitivity may be overcome by replacing the ordinary paper backing by an electrically-conducting material, such as a metal or a paper treated with carbon or certain silver salts. Such replacement results in one or more of the following disadvantages: (1) the backing is more expensive, (2) the backing is not easily coated with standard web coating machines, (3) the backing is not compatible with the photoconducting coating, (4) the backing is too rigid or inflexible for many uses, and (5) the color of the backing is objectionable.

An object of this invention is to provide improved electrophotographic recording elements for electrostatic printing and improved methods of electrostatic printing including using the improved recording elements of the invention.

Another object is to provide improved recording elements for electrostatic printing which recording elements are cheap, flexible and easily prepared in standard web coating machines.

A further object is to provide improved electrophotographic recording elements for electrostatic printing whose printing characteristics are substantially independent of the humidity in which it is stored prior to use.

25 In general, the recording elements of the invention comprise a photoconducting stratum contiguous with a substratum comprising a particulate semiconductor dispersed in a binder, said substratum having a short dark decay relative to the dark decay of said photoconducting stratum. By placing a substratum of the type described contiguous with the photoconducting stratum, the photoconducting stratum is relatively independent of the characteristics of the backing during charging and exposure. It is believed that at low humidities as well as high humidities, the electric field at the time of charging appears across the backing, stratum and substratum. But, because of the relatively short decay of the substratum, a relaxation occurs in the substratum strengthening the effective electric field across the photoconducting stratum. Also, improved lateral conductivity of the substratum provides more uniform effective electric fields across the photoconducting stratum.

An example of a recording element of the invention comprises a paper sheet having coated thereon a substratum including a particulate semiconducting zinc oxide dispersed in a cellulose acetate resin and, coated thereon, a photoconducting stratum having a long dark decay relative to the dark decay of said substratum and including a particulate photoconducting zinc oxide in a silicone resin. The invention includes recording elements comprising the stratum and substratum described above both with or without a backing.

The foregoing objects and other advantages are more fully described in the following detailed description when read in conjunction with the accompanying drawing in which:

Figure 1 is a sectional, elevational view of a typical recording element according to the invention.

Figure 2 is a partially-schematic, sectional view of an apparatus for producing a blanket electrostatic charge 60 upon a recording element produced by the method of the invention.

Figure 3 is a partially-sectional, elevational view of an apparatus for projecting a light to form a contact image upon the charged recording element of Figure 2, and

Figure 4 is a sectional view of an apparatus for developing an electrostatic image upon the recording element produced in Figure 3, and

Figure 5 is a family of curves illustrating the dark decays of combinations of various zinc oxides and various vehicles.

Similar reference characters are applied to similar structures throughout the drawings.

A detailed example for preparing and using an electro-photographic recording element in accordance with the present invention will now be given.

*Example 1.*—Referring to Figure 1, a recording element according to the invention is prepared as follows: a first mixture is prepared by dissolving 20 grams of soluble casein in 200 grams of water and 1 cc. of 28% aqueous ammonium hydroxide. Then about 50 grams of semiconducting zinc oxide such as AZO ZZZ-33 marketed by the American Zinc Sales Company, 420 Lexington Avenue, New York, N.Y., is dispersed in the solution. This dispersion is coated on a paper backing 19 by any conventional coating process, and the coating dried thereby producing a substratum 21 on the paper backing 19.

A second coating mixture is prepared by mixing 80 grams of 60% solution of silicone resin in xylene, such as GE SR-82 marketed by the General Electric Company, Silicone Products Division, Waterford, New York, 106 grams of toluene, and 120 grams of white photoconducting zinc oxide, such as Florence Green Seal-8 French Process Zinc, marketed by the New Jersey Zinc Company, Palmerton, Pa. The mixture is ball-milled to a smooth uniform consistency and is applied to the surface of the substratum 21 and then dried thereby producing a photoconducting stratum 23 upon the semiconducting substratum 21. Any standard coating technique may be used to produce the foregoing substratum 21 and stratum 23 such as flowing, spraying, dipping, spin coating or brushing on.

Upon drying, the recording element is ready for use. It may be stored for long or short periods of time in a hot or cold storage wherein the humidity is high or low. Regardless of the humidity of the storage conditions, the recording element will produce good prints.

The recording elements of the invention may be used for electrostatic printing by any of the methods described in the Young and Greig publication, op. cit. By way of example and referring to Figure 2, the recording element of Example 1 may be utilized in an electrostatic printing process according to the following steps. The recording element is placed with the backing 19 upon a grounded metal plate 25 and in darkness, an electrostatic charging device 61 passed over the photoconducting stratum 23 to provide an electrostatic charge thereon. The charging device 61 may comprise an array of fine wires 53 mounted near the grounded metal plate 25. A source of D.C. voltage is connected between the wires 53 and the grounded plate 25 to provide a negative charge on the wires with respect to grounded plate 25. The voltage should be sufficiently high to cause a corona discharge adjacent the wires. It is preferred to apply about -6000 volts with respect to ground to the wires 53 when charging the surface of the recording element of the example. The surface of the recording element passing under the charging device 61 becomes charged negatively with the preferred voltage applied. The apparatus and process may produce a blanket positive charge if the polarity of the wires 53 is positive with respect to the grounded plate 25.

The next step in the process is to discharge selected areas of the charged surface of the recording element in order to produce an electrostatic image thereon. Referring to Figure 3, this may be accomplished by placing a photographic transparency 61 upon the charged surface 23 and exposing to light derived, for example, from a lamp 59 in the manner of conventional contact printing. An exposure of about 1 second from a 100 watt tungsten lamp about 24 inches from the recording element for a normal density photographic transparency has been found to be adequate. The light image may be produced by any of the ordinary photographic processes as by projection, contact, or reflex. Any type

of electromagnetic radiation may be used provided a portion falls within the spectral sensitivity of the photoconducting stratum 23. In Example 1 visible blue and ultra-violet light may be used. For other photoconducting strata, visible light, infra-red, or ultra-violet may be used.

Wherever the light strikes the surface of the photoconducting stratum 23, the electrostatic charge thereon is reduced or removed. This leaves an electrostatic image or pattern of charges corresponding to the non-illuminated areas of the light image.

The electrostatic image may be stored for a time if desired. Ordinarily the next step is to develop the electrostatic image with a finely-divided developer substance 15 such as a finely-divided powder or an ink mist. Referring to Figure 4, development of the electrostatic image is preferably accomplished by maintaining the recording element in darkness and passing a developer brush 55 containing a developer powder across the surface of photoconducting stratum 23 bearing the electrostatic image. Areas 27 of developer powder are deposited on those areas of the surface retaining an electrostatic charge. The developer brush comprises a mixture of magnetic carrier particles, for example powdered iron, and the developer powder. The mixture is secured in a magnetic field by a magnet 57 to form a developer brush.

A preferred carrier material for the developer mix consists of "alcoholized iron," that is, iron particles free from grease and other alcohol soluble impurities. These 30 iron particles are preferably relatively small in size, being in their largest dimension about .002" to .008". Satisfactory results are also obtained using a carrier consisting of iron particles of a somewhat wider range of sizes from about .001" to .020".

35 A preferred developer powder may be prepared as follows: A mixture comprising 200 grams of 200 mesh Piccolastic resin 4358 (an elastic thermoplastic resin composed of polymers of styrene, substituted styrene and its homologs) marketed by the Pennsylvania Industrial Company, Clairton, Pa., 12 grams of Carbon Black G, marketed by the Eimer and Amend Co., New York, N.Y., 12 grams of spirit Nigrosine S.S.B. marketed by the Allied Chemical and Dye Co., New York, N.Y., and 8 grams of Iosol Black marketed by the Allied Chemical and Dye Co., New York, N.Y., are thoroughly mixed 40 in a stainless steel beaker at about 200° C. The mixing and heating should be done in as short a time as possible. The melt is poured into a brass tray and allowed to cool and harden. The hardened mix is then broken up and ball-milled for about 20 hours. The powder is screened 45 through a 200 mesh screen and is then ready for use as a developer powder. This powder takes on a positive electrostatic charge when mixed with glass beads or iron powder. It therefore develops an electrostatic image composed of negative charges. Two to four grams of the developer powder and 100 grams of the magnetic carrier material are blended together giving the preferred developer mix. Other ratios may be used.

The developer powder may be chosen from a large 60 class of materials. The developer powder is preferably electrically-charged to aid in the development of the electrostatic latent image. The powder may be electrically-charged because the powder (1) is electroscopic, or (2) has interacted with other particles with which it is 65 triboelectrically active or (3) has been charged from an electric source such as a corona discharge. Examples of suitable developer powders are powdered zinc, powdered copper, carbon, sulfur, natural and synthetic resins or mixtures thereof.

The developer powder may be applied to the electrostatic image in other ways, for example, it may be dusted on to the image, or it may be mixed with glass beads or other suitable carrier particles, the mixture then brought 70 into contact with the surface of the photoconducting stratum. The beads serve merely as a temporary carrier,

releasing the powder particles upon contact with the charged surface.

The type of developer powder described is a positively-charged powder and will adhere readily to negatively charged areas of the electrostatic image. In the developed image described, the developed areas of the image correspond to the non-illuminated portions of the light image. If the photoconducting stratum is charged positively, and the same steps are carried through as above described, a reverse image is obtained. If a negatively charged powder is used in place of the positively charged powder, then a reverse image is obtained in the first case and a positive image is obtained in the alternative case.

The developed image 27 is now fixed to the photoconducting stratum 23. If the developer powder or the vehicle in the photoconducting stratum 23 has a relatively low melting point, the developed image may be fixed by heating, for example with an infra red lamp, to fuse the powder to the surface. Sulfur or synthetic thermoplastic resin powders may be fixed in this way. Alternatively, the developed image 27 may be pressed into the stratum 23. Another method of fixing the developed image 27 is to apply a thin coating of a solvent for the material of the developed image 31. The solvent softens the developer powder particles and causes them to adhere to one another and to the photoconducting stratum 23. Alternatively, a solvent may be used to soften the photoconducting stratum 23 and cause the developed image to adhere thereto. Upon standing, and preferably with the application of a slight amount of heat, the solvent is evaporated from the recording element.

Prints made with the recording element of Example 1 which has been stored just prior to use at normal or above normal humidity conditions by the foregoing printing procedure are comparable with those made on a similar recording element having no substratum 21. If the two recording elements are thoroughly dried just prior to use, as by heating for five minutes at about 150° C., the recording element without the substratum 21 blanks out entirely or prints only in patches, whereas the recording element of the invention still gives good prints.

Figure 5 illustrates the difference in dark decays between the photoconducting stratum 23 and the substratum 21 of the recording element of Example 1. The photoconducting coating composition (Florence Green Seal-8, toluene and silicone) is coated on aluminum foil and dried. The coating is then maintained in darkness at a constant controlled humidity for about 2 hours, then charged as set forth above. The surface voltage was measured continuously after charging. The curves 71 and 73 represent the surface voltage with respect to time for this coating at about 15% relative humidity and 90% relative humidity respectively at about 70° F.

The substratum coating composition (AZO ZZZ-33, water and casein) was similarly coated on aluminum foil, dried and charged. The curve 75 represents the surface voltage with respect to time for this substratum coating at about 5% relative humidity and about 70° F. Above 50% relative humidity, no surface voltage is detected. Note that, although the charging is the same, the charge is dissipated extremely rapidly in the case of the substratum coating as shown by the curve 75 compared with the photoconducting coating as shown by the curves 71 and 73. The combination of AZO ZZZ-33 and silicone resin under similar conditions is illustrated by the curve 77.

Example 2.—A thin porous paper is impregnated with the first coating mixture of Example 1 and dried. The second coating mixture of Example 1 is then applied to one side of this impregnated sheet and dried. The substratum which comprises the impregnated paper acts as a floating ground or a conducting link to ground during charging. Under dry humidity conditions the recording element is not attracted to the ground plate (does not "lock down") during charging and will print in humidity

conditions where a recording element without a semiconducting substratum completely blanks out.

Example 3.—A thin relatively porous paper sheet, such as a manifold bond, is filled with a semiconducting zinc oxide powder. This can be done by rubbing or brushing a thin suspension or paste of the semiconducting zinc oxide into the interstices of the paper and then removing the vehicle by drying. The preferred method however, is to add the zinc oxide to the pulp at the time the paper is made, for example, by one of the conventional procedures used for making a filled paper. The filled sheet is then coated in the usual way with the second or photoconductive coating mix of Example 1 and dried.

The binder of the stratum coating penetrates into the filled paper backing yielding a substratum comprising paper impregnated with zinc oxide and vehicle similar to the recording element of Example 2. Thus, the stratum and substratum may comprise the same vehicle and may be prepared by a single coating step. This recording element prints the same as the recording element in Example 2.

Example 4.—A paper sheet is coated with a substratum coating mixture comprising 10 grams of cellulose acetate such as Eastman Kodak No. 4644 Vis. 3, marketed by the Tennessee Eastman Corporation, Kingsport, Tennessee; 200 grams of acetone and 50 grams of AZO ZZZ-33 zinc oxide marketed by the American Zinc Sales Co., and dried, producing a substratum on the paper backing. The substratum is then coated with the second coating mix of Example 1 producing a photoconducting stratum upon the substratum.

The recording elements of the examples utilize a semiconducting zinc oxide and a photoconducting zinc oxide. In the research work to develop an electrophotographic recording element described in the Young and Greig publication, *op. cit.*, it was noted that several of the zinc oxides tried for making recording elements, did not print or printed very poorly. Most of these were American Process zinc oxides produced directly from the zinc ore. Probe measurements, such as those illustrated in Figure 5, of the equivalent surface voltage immediately after charging the photoconducting stratum in the dark showed little or no retention of the surface charge. It is believed that the dark decay of the inoperative strata, even when comprised of a highly insulating vehicle, such as silicone resin, is too rapid for the strata to be operative in the ordinary electrostatic printing process. However, such a coating is ideal for the substratum of the present invention. These zinc oxides in any binder or as a filler in a base sheet itself provide a smooth support for the photoconducting stratum in the electrostatic printing process. The recording elements of the invention are relatively independent of moisture content in the supporting sheet or backing and one may omit the backing completely if they are sufficiently strong.

The semiconducting zinc oxides are identical in appearance with the so-called photoconducting zinc oxides. Several tests have been devised to distinguish the zinc oxides which are useful in the photoconducting stratum from the semiconducting zinc oxides that are useful in the semiconducting substratum as follows:

I. Prepare a zinc oxide-vehicle mix as described for the second coating mixture of Example 1. Coat the mixture on aluminum foil and dry. Then attempt to produce a print as described in Example 1. A zinc oxide that produces a layer that prints is useful in the photoconducting stratum. A zinc oxide that does not print or prints poorly is useful in the substratum.

II. Prepare a zinc oxide-vehicle mix as described for the second coating mixture of Example 1. Coat the mixture on aluminum foil and dry. Then cool to liquid nitrogen temperatures (about -60° C.) and irradiate with 3650 Å. radiation. A printable stratum exhibits a lavender or orange luminescence. A non-printable or

poorly printable stratum exhibits a green or yellow luminescence.

III. The zinc oxide sample is fired in hydrogen at about 1000° C. for about 10 minutes. The sample is cooled and irradiated with 3650 A. radiation. The zinc oxides which produce printable strata luminesce brightly whereas the zinc oxides which produce non-printable or poorly printable strata luminesces weakly or not at all.

The table compiles the results of the three tests on typical commercially available zinc oxides and indicates the correlation between these tests. The zinc oxides marked "v" in column I may be used in the photoconducting stratum while the zinc oxides marked "o" may be used in the semiconducting substratum.

Table

| Zinc Oxide                                         | I (a) | II (b)       | III (c)       |
|----------------------------------------------------|-------|--------------|---------------|
| Mallinckrodt:<br>AR WXAV-1                         | v     | lavender     | bright green. |
| AR WYEB                                            | v     | or.-lavender | Do.           |
| Y-1000                                             | v     | orange       | grey green.   |
| Eagle-Picher:<br>USP                               | v     | lavender     | bright green. |
| 109                                                | v     | do           | Do.           |
| 310                                                | v     | do           | Do.           |
| 417                                                | o     | green        | faint green.  |
| 730                                                | o     | yellow       | dead.         |
| AZO:<br>22                                         | o     | green        | nearly dead.  |
| 33                                                 | v     | do           | Do.           |
| 44                                                 | v     | do           | Do.           |
| 66                                                 | v     | lavender     | bright green. |
| Spec. Pure:<br>N.J. Zinc <sup>4</sup>              | v     | do           | Do.           |
| Spex Standard <sup>5</sup>                         | v     | do           | Do.           |
| Johnson-Matthey <sup>6</sup>                       | v-x   | yellow       | Do.           |
| Miscellaneous:<br>E. and A. <sup>7</sup> wet proc. | v     | lavender     | Do.           |
| N.J.Z. Spec. No. 3                                 | x     | yellow       | dull green.   |
| Florence Green Seal (standard)                     | v     | lavender     | bright green. |

(a)=printability, v=good, x=lower contrast, o=does not print.  
(b)=luminescence at liquid nitrogen temperature in silicone resin:

3650 A. exciting radiation.

(c) luminescence at room temperature under 3650 A. lamp after firing

at 1000° C. in hydrogen.

<sup>1</sup> Mallinckrodt Chemical Works, New York, N.Y.

<sup>2</sup> Eagle Picher Sales Co., Philadelphia, Pa.

<sup>3</sup> American Zinc Sales Co., New York, N.Y.

<sup>4</sup> New Jersey Zinc Co., Palmerton, Pa.

<sup>5</sup> Spex Industries, Queens Village 27, N.Y.

<sup>6</sup> Johnson, Matthey and Co., 73 Hatton Garden, London, England.

<sup>7</sup> Eimer and Amend Co., Division of Fisher Scientific Co., New York

14, N.Y.

While the reason for this improvement is not fully understood, the following explanation is offered to aid in understanding the improvement. In the recording elements of the invention, the substratum 21 has a very rapid dark decay and appears to act as a sink or floating ground which has enough lateral and transverse conductivity to permit developing adequate uniform electric field across the photoconducting stratum just prior to exposure. The photoconducting stratum has a very long decay with the result that the electric fields from the charging apparatus are more effectively utilized.

Other semiconducting materials which have shown the same effect when substituted for the semiconducting zinc oxide above are:

- (1) Stannic oxide (Eimer and Amend Company, Catalogue No. T-148, New York, N.Y.)
- (2) Zinc oxide AZO ZZZ-11 (American Zinc Sales Company, New York, N.Y.)
- (3) Zinc oxide AZO ZZZ-22 (American Zinc Sales Company, New York, N.Y.)
- (4) Zinc oxide AZO ZZZ-44 (American Zinc Sales Company, New York, N.Y.)
- (5) Zinc oxide No. 720 (Eagle Picher Sales Company, Philadelphia, Pa.)
- (6) Titanium dioxide R-510 and LO-CR (E. I. du Pont de Nemours, Wilmington, Delaware)
- (7) Basic lead carbonate—Catalogue No. 74 C.P. (Eimer and Amend Co., New York 14, N.Y.)

Any of the foregoing materials may be substituted for the semiconducting zinc oxides of the examples. It is

only necessary that the material in combination with a vehicle produce a substratum having a short dark decay relative to the dark decay of the photoconducting stratum. For high speed printing, the thickness and composition of the substratum is preferably adjusted to possess the shortest dark decay possible.

The materials of the foregoing paragraphs are operative when dispersed in a wide range of binders to oxide ratios as an undercoat or impregnation material. One may use small amounts of binder in ratios up to one part by weight of binder to 2½ parts by weight of semiconducting zinc oxide. The upper limit is set by loose oxide particles interfering with the photoconducting coating, the lower limit is set by the ratio at which conductivity of the substratum is too low for the desired application.

The requirements for the vehicle of the substratum are much less stringent than for the vehicles used in the photoconducting stratum. When the substratum is used

20 as a film or coating on the flexible recording element, the substratum should of course, have the necessary flexibility, adhesions, shelf-life, desired in the composite sheet. If the substratum is to be overcoated with a photoconducting stratum, it is desirable that the vehicle in the substratum have a different solvent solubility than that

25 of the vehicle for the photoconducting stratum, so that the photoconducting stratum may be applied without undue mixing or dissolution in the two strata. Many of the desired properties of the substratum can be obtained by the use of additives or modifiers in the mix. For example, plasticizers may be added to gain flexibility, surface active agents may be added to gain adhesive characteristics, toughening agents may be added to gain strength. The vehicle for the substratum may be a

30 synthetic or natural resin or wax and may be organic solvent or water soluble. Examples of suitable vehicles are cellulose acetate, cellulose acetate butyrate, polyvinyl acetate, polyvinyl chloride, polyvinyl chloride acetate, shellac, rosin, carnauba wax, beeswax, paraffin, polyethylene glycol, casein, hydroxyethyl cellulose, carboxymethyl cellulose or gum.

The photoconducting stratum 23 must be a material which exhibits a substantial change in electrical conductivity upon exposure to light, such that an electrostatic

45 charge stored on the surface thereof may be discharged. The photoconducting stratum 23 determines the spectral response, the speed of response and the contrast characteristic of the recording element. By a proper choice of materials for the photoconducting stratum 23, any spectral response, speed of response or contrast characteristic

50 over a wide range may be obtained. Many different powdered photoconductors may be used in the photoconducting stratum in place of the white zinc oxide. For example, one may use dye-sensitized white zinc oxide, cadmium-zinc sulfide, or panchromatically sensitive or buff zinc oxide, as described in U.S. Patents 2,727,807 and 2,727,808 to S. M. Thomsen. The photoconducting stratum may be any of the photoconducting coatings described in the Young and Greig publication, *ibid.*

55 The vehicle for the photoconducting stratum 23 is essential and may comprise any one of a number of substances which are film-forming and electrically-insulating. In place of a silicone resin, one may use any of the following vehicles: polystyrene, polyvinyl acetate, copolymers of vinyl chloride-acetate, cellulose ethers, cellulose esters, methyl and ethyl cellulose, cellulose nitrate, shellac, paraffin wax, and carnauba wax.

60 The photoconductor may be suspended in the vehicle in any one of several ways. The simplest way is to disolve the vehicle in an organic solvent capable of effecting solution and then mixing in the powdered photoconductor. Alternatively, the photoconductor may be dry blended, as by kneading with the vehicle heated to a sufficiently high temperature to render it plastic.

65 The proportion of photoconductor to vehicle in the

photoconducting stratum may vary over a very wide range. The preferred ranges are about 50% to 90% by weight of photoconductor to about 50% to 10% by weight of vehicle. The optimum proportion depends upon the nature of the photoconductor, the nature of the vehicle and the results that are desired.

The examples describe recording elements including a paper backing which provides a mechanical support for the stratum and substratum. The backing may be any web material but is preferably cellulosic such as ordinary paper or cellophane. If the stratum and substratum are sufficiently strong, the backing may be omitted.

There have been described improved electrophotographic recording elements for electrostatic printing and improved methods of electrostatic printing utilizing the recording elements of the invention. The recording elements of the invention are cheap, easily prepared in standard web coating machines, flexible and are substantially insensitive to the relative humidity in which they are stored prior to use in an electrostatic printing process.

What is claimed is:

1. An electrophotographic recording element including a photoconducting insulating stratum comprising particles of photoconducting zinc oxide dispersed in an electrically-insulating, solid, film-forming vehicle in contact with a semiconducting substratum comprising particles of a semiconducting material selected from the group consisting of semiconducting zinc oxide, stannic oxide, titanium dioxide and basic lead carbonate, in a solid, film-forming vehicle, said photoconducting stratum having a long dark decay relative to the dark decay of said substratum, the weight ratio of photoconducting zinc oxide to vehicle in said stratum being between 50/50 and 90/10, and the vehicle being present in said substratum in proportions up to one part by weight vehicle to two and a half parts by weight semiconducting material.

2. A recording medium according to claim 1 wherein said stratum and substratum are self-supporting.

3. A recording element according to claim 1 wherein said substratum is coated upon a support.

4. A recording element according to claim 1 wherein said substratum is impregnated into a porous support.

5. An electrophotographic recording element comprising a web of cellulosic material, a semiconducting substratum comprising particles of a semiconducting material selected from the group consisting of semiconducting zinc oxide, stannic oxide, titanium dioxide, and basic lead carbonate, dispersed in a solid film-forming vehicle upon a surface of said web, and a photoconducting insulating stratum comprising particles of photoconducting zinc oxide dispersed in an electrically-insulating, solid, film-forming vehicle upon said substratum, said photoconducting stratum having a long dark decay relative to the dark decay of said substratum, the weight ratio of photoconducting zinc oxide to vehicle in said stratum being between 50/50 and 90/10, and the vehicle being present in said substratum in proportions up to one part by weight vehicle to two and a half parts by weight semiconducting material.

6. An electrophotographic recording element including a photoconducting insulating stratum comprising particles of photoconducting zinc oxide dispersed in a water-insoluble, electrically-insulating, solid, film-forming vehicle upon a semiconducting substratum having a short dark decay relative to the dark decay of said photoconducting stratum and comprising particles of a semiconducting material selected from the group consisting of semiconducting zinc oxide, stannic oxide, titanium dioxide, and basic lead carbonate, dispersed in a water-soluble, solid, film-forming vehicle, the weight ratio of photoconducting zinc oxide to vehicle in said stratum being between 50/50 and 90/10; and the vehicle being present in said substratum in proportions up to one part by

5 weight vehicle to two and a half parts by weight semiconducting material.

7. An electrophotographic recording element according to claim 6 wherein said semiconductor comprises zinc oxide.

8. An electrophotographic recording element comprising a paper support sheet, a semiconducting substratum including a particulate semiconducting zinc oxide dispersed in a cellulose acetate vehicle upon a surface of 10 said support sheet and, upon said substratum, a photoconducting insulating stratum having a long dark decay relative to the dark decay of said substratum and comprising a particulate photoconducting zinc oxide dispersed in a silicone resin vehicle, the weight ratio of photoconducting zinc oxide to vehicle in said stratum being between 50/50 and 90/10, and the vehicle being present in said substratum in proportions up to one part by weight vehicle to two and a half parts by weight semiconducting zinc oxide.

15 20 9. An electrophotographic recording element comprising a paper support sheet, a semiconducting substratum including a particulate semiconducting zinc oxide dispersed in a casein vehicle upon a surface of said support sheet and, upon said substratum, a photoconducting 25 insulating stratum having a long dark decay relative to the dark decay of said substratum comprising a particulate photoconducting zinc oxide dispersed in a silicone resin vehicle, the weight ratio of photoconducting zinc oxide to vehicle in said stratum being between 50/50 30 and 90/10, and the vehicle being present in said substratum in proportions up to one part by weight vehicle to two and a half parts by weight semiconducting zinc oxide.

35 10. A print receiving element comprising a paper sheet; 40 a semiconducting substratum upon a surface of said sheet, said substratum comprising a major proportion of particles of semiconducting zinc oxide and a minor proportion of a casein binder, said binder being present in said substratum in proportions up to one part by weight binder to two and a half parts by weight semiconducting zinc oxide; and a photoconducting insulating stratum upon said substratum, said stratum comprising a major proportion of particles of photoconducting zinc oxide and a minor proportion of a silicone resin vehicle, said vehicle being present in said stratum in proportions between 50 and 90 weight parts photoconducting zinc oxide and between 10 and 50 weight parts vehicle, said photoconducting stratum having a long dark decay relative to the dark decay of said substratum.

45 50 11. A print receiving element comprising a paper sheet; 55 a semiconducting substratum upon a surface of said sheet, said substratum comprising a major proportion of particles of semiconducting zinc oxide and a minor proportion of a casein binder, said binder being present in said substratum in proportion of one part by weight binder to two and a half parts by weight semiconducting zinc oxide; and a photoconducting insulating stratum upon said substratum, said stratum comprising a major proportion of particles of photoconducting zinc oxide and 60 a minor proportion of a silicone resin vehicle, said vehicle being present in said stratum in proportions of 100 weight parts photoconducting zinc oxide and 40 weight parts vehicle, said photoconducting stratum having a long dark decay relative to the dark decay of said substratum.

65 12. A print receiving element comprising a paper sheet; 70 a semiconducting substratum upon a surface of said sheet, said substratum comprising a major proportion of particles of semiconducting zinc oxide and a minor proportion of a cellulose acetate binder, said binder being present in said substratum in proportions up to one part by weight binder to two and a half parts by weight semiconducting zinc oxide; and a photoconducting insulating stratum upon said substratum, said stratum comprising a major proportion of particles of photoconducting zinc oxide and a minor proportion of a silicone resin vehicle,

said vehicle being present in said stratum in proportions between 50 and 90 weight parts photoconducting zinc oxide and between 10 and 50 weight parts vehicle, said photoconducting stratum having a long dark decay relative to the dark decay of said substratum.

13. A print receiving element comprising a paper sheet; a semiconducting substratum upon a surface of said sheet, said substratum comprising a major proportion of particles of semiconducting zinc oxide and a minor proportion of a cellulose acetate binder, said binder being present in said substratum in proportions of one part by weight binder to two and a half parts by weight semiconducting zinc oxide; and a photoconducting insulating stratum upon said substratum, said stratum comprising a major proportion of particles of photoconducting zinc oxide and a minor proportion of a silicone resin vehicle, said vehicle being present in said stratum in proportions of 100 weight parts photoconducting zinc oxide and 40 weight parts vehicle, said photoconducting stratum having a long dark decay relative to the dark decay of said substratum.

## References Cited in the file of this patent

## UNITED STATES PATENTS

|           |           |                |
|-----------|-----------|----------------|
| 2,297,691 | Carlson   | Oct. 6, 1942   |
| 2,427,700 | Atkinson  | Sept. 23, 1947 |
| 2,476,800 | Blackburn | July 19, 1949  |

|           |                 |               |
|-----------|-----------------|---------------|
| 2,554,017 | Dalton          | May 22, 1951  |
| 2,613,301 | Dubar et al.    | Oct. 7, 1952  |
| 2,662,957 | Eisler          | Dec. 15, 1953 |
| 2,664,044 | Dalton          | Dec. 29, 1953 |
| 2,735,784 | Greig et al.    | Feb. 21, 1956 |
| 2,761,849 | Coler           | Sept. 4, 1956 |
| 2,798,959 | Moncrief-Yeates | July 9, 1957  |
| 2,825,814 | Walkup          | May 4, 1958   |
| 2,862,815 | Sugarmen et al. | Dec. 2, 1958  |
| 2,887,632 | Dalton          | May 14, 1959  |
| 2,901,348 | Dessauer et al. | Aug. 25, 1959 |

## FOREIGN PATENTS

|           |           |               |
|-----------|-----------|---------------|
| 449,303   | Canada    | June 22, 1948 |
| 1,022,091 | Germany   | Jan. 2, 1958  |
| 157,101   | Australia | June 16, 1954 |

## OTHER REFERENCES

|    |                                                                                                  |
|----|--------------------------------------------------------------------------------------------------|
| 20 | Semi-Conductor Abstracts, vol. III, 1955 issue, pp. 85-88.                                       |
| 25 | The Condensed Chem. Dict., Reinhold (1956), p. 727 "Methy Violet," and p. 322, "crystal violet." |
|    | Vartanian: Acta Physiochemica U.R.S.S., vol. XXII, No. 2, pp. 201-224 (1947).                    |
|    | Cochran: Batelle Tech. Review, vol. 3, No. 7, pp. 71-74.                                         |
|    | Wainer: Photographic Engineering, vol. 3, No. 1, pp. 12-22 (1952).                               |